

## UNITED STATES PATENT OFFICE

1,977,404

## VEGETABLE PROTEIN GLUE

Russell G. Peterson, Tacoma, Wash., assignor to  
George H. Osgood, Tacoma, Wash.No Drawing. Application July 29, 1931.  
Serial No. 553,885

4 Claims. (Cl. 87—17)

The art of making glues from vegetable flours made from protein-bearing materials, such as soya bean, peanut, cottonseed, linseed, castor bean, and the like, has been known and has been largely used on account of the cheapness of the materials, but difficulty has been encountered in making such a glue which does not require the constant attention of an experienced glue-mixer on account of the other materials formerly necessary to make a usable glue, such as caustic soda, silicate of soda, carbon bisulphide, and the like, which cannot be put into the glue itself in the dry state but must be carefully measured and mixed after the soya bean flour, or other constituents, have been mixed with water.

I have found that such glues can be made more highly water-resistant if they are formed with a water-soluble product of cellulose, namely viscose, and that they do not require the skill-  
ful attention of an expert in their preparation.

Since these several vegetable meals are all slightly acid and since such acid content would separate the cellulose in the viscose used, to make an insoluble compound, I neutralize the meal before it is used in making the glue. This neutralization may be effected by the suitable use of any soluble sodium salt, or any alkaline earth materials.

To this neutralized vegetable flour is added a water-soluble product of cellulose, namely, viscose, in the proportion of about 25 to 40 parts of the viscose to 100 parts of the neutralized meal. This viscose contains an excess of caustic in order that it will be retained in liquid condition, and this excess of caustic acts as a solvent for the meal, while the cellulose in the viscose acts as a means of increasing its water-resistance.

The viscose is prepared under standard direc-

tions such as those published by Cross & Bevins, using rayon pulp, or other high grade wood pulp, as a base. Other suitable materials, such as cotton straw, can be used if desired.

The wood, being glued, is slightly acid and when such a glue, as above described, is applied to the wood, the acids in the wood itself neutralize the caustic of the glue and slightly acidifies the glue line, which is then highly water-resistant.

The glues are prepared in an aqueous medium, in suitable proportions, about 250 parts of water to 100 parts of neutralized flour being usually found sufficient.

Having described my invention, I claim:—

1. An adhesive composition comprising an aqueous mixture of a neutralized protein-bearing vegetable meal, with cellulosic viscose containing an excess of alkali as a dispersing medium for the meal.

2. An adhesive composition comprising an aqueous mixture of 100 parts of neutralized protein-bearing meal, with 25 to 40 parts of cellulosic viscose containing an excess of alkali as a dispersing medium for the meal.

3. An adhesive composition comprising a neutralized vegetable protein-bearing meal as a base; with cellulosic viscose containing an excess alkalinity which is used as a solvent for the meal and as a water-proofing agent for the compound.

4. An adhesive composition comprising a neutralized vegetable protein-bearing meal and cellulosic viscose containing an excess of alkali, which acts as a dispersing medium for the meal, and which, when applied between the layers of acid wood, is acted on by the acid in the wood to neutralize the excess caustic of the compound to form a water-resistant glue line.

RUSSELL G. PETERSON.

40

95

45

100

50

105

55

110